

A. S. DWIGHT.

## SINTERING AND SMELTING ORE.

APPLICATION FILED MAR. 31, 1910, RENEWED JUNE 15, 1916.

1,215,635.

Patented Feb. 13, 1917.



## Witnesses

B. G. Bram  
S. Jay Teller

Inventor  
Arthur S. Dwight  
By H. A. Bliss  
Attorney

# UNITED STATES PATENT OFFICE.

ARTHUR S. DWIGHT, OF NEW YORK, N. Y.

## SINTERING AND SMELTING ORE.

1,215,635.

Specification of Letters Patent. Patented Feb. 13, 1917.

Application filed March 31, 1910, Serial No. 552,578. Renewed June 15, 1916. Serial No. 103,863.

To all whom it may concern:

Be it known that I, ARTHUR S. DWIGHT, a citizen of the United States, residing at New York, in the county of New York and State of New York, have invented certain new and useful Improvements in Sintering and Smelting Ores, of which the following is a specification, reference being had thereto in to the accompanying drawing.

10 This invention relates to improvements in processes for treating ores, particularly those which are susceptible of a desulfurizing or kindred treatment and a sintering treatment, either simultaneously or successively, and of being subsequently reduced by smelting or a similar operation.

15 It will be understood that my improved process is not limited to the treatment of ores normally containing a combustible element, such as sulfur, but may be used for the treatment of iron or other ores to which a combustible element, such as carbon, has been artificially added.

20 The process is similar in some respects to that set forth in my co-pending application entitled Desulfurizing and smelting ores, filed June 25, 1908, Serial No. 440,404. I do not, therefore, herein claim the broader features of the process set forth in the said application.

25 The essential steps of the process to which my invention relates can be carried out in apparatus of any of a number of forms. In the accompanying drawings I have shown for purposes of illustration one form of apparatus adapted for use in the practice of my invention.

30 Of the drawings—

35 Figure 1 is a side view partly in elevation and partly in vertical section and shows an apparatus adapted to be used in carrying out my improved process.

40 Fig. 2 is a plan view, a part being shown in cross section along the line 2—2 of Fig. 1.

45 Fig. 3 is a fragmentary cross sectional view taken along the line 3—3 of Fig. 2.

50 It will be understood that the apparatus presented in the drawings is illustrated more or less conventionally but in such a way that the essential parts of the process and of the apparatus may be readily understood by those skilled in the art. Generally

considered, the process can be regarded as comprising two stages, and the devices illustrated for carrying out the process can be considered as made up of two main parts.

55 The apparatus indicated by A is especially adapted for treatment of sulfid ores, such as copper sulfid, although it is to be understood that the invention is not limited to the treatment of material of any particular type.

60 The apparatus indicated by A comprises a traveling conveyer 1. This conveyer 1 may be of any desired type, but I prefer to use a conveyer comprising a series of pans, buckets or pallets 2. These pallets are provided with perforated bottoms and side walls perpendicular to the bottoms. Wheels 3, 3 are provided for each pallet and these wheels are adapted to engage with and be supported by the tracks 4 and 5. The pallets are adapted to align with each other at the upper part of the conveyer to form a continually moving tray or platform supported by the track 4. At its forward end the track 4 is overlapped by the track 5 in such a way that a pallet on passing around the curved end of the track 4 will be engaged by the overlapping curved end of the track 5 on which it will be carried by gravity to the continually rotating wheel 6. This wheel is provided with teeth adapted to engage the wheels of the pallets and to thus carry the inverted pallets upward onto the track 4.

65 A hopper 7 is provided for the reception of material and serves to direct the material onto the moving conveyer in a stream or layer of substantially uniform thickness.

70 8 represents an air box provided with means for exhausting the air therefrom. The top of this box is formed by the perforated bottoms of the moving pallets and consequently as air is withdrawn from the box by the exhausting means, it is drawn in through the perforations in the pallet bottoms.

75 When there is a layer of ore on the pallets then the air will be drawn downward through the interstices between the ore fragments.

80 9 represents an igniting apparatus which may be of any preferred form, such as a gas pipe perforated to provide a series of gas jets across the top of the ore mass or a con-

ductor and burner for oil. The stream or layer of ore delivered from the hopper 7 passes under the apparatus 9, and the combustible elements, such as sulfur or carbon 5 contained in the ore charge, are ignited.

It is not necessary to here describe in detail the various successive steps incident to the sintering of the ore, as these are fully described in patents issued to A. S. Dwight 10 and R. L. Lloyd, among them being Patent 882,517 and Patent 882,518. For the purposes of the present description, it is sufficient to say that the ore moves along with the conveying apparatus 1, and that the 15 combustion started by the igniting device 9 moves gradually downward through the stream or layer of ore under the influence of the downward draft of air caused by the exhausting device connected with the air 20 box 8. The combustion is entirely supported by the combustible elements, such as sulfur contained in the ore itself, and the lines of combustion move downward until they reach the bottom of the layer. The 25 heat generated by the combustion causes certain constituent elements of the ore mass to melt and unite the layer into a homogeneous coherent porous cake. The rate of motion of the conveyer 1, and the thickness of the 30 layer of ore are so regulated that the desulfurizing and sintering processes will be completed when the moving layer reaches the point 10. As each pallet reaches the 35 point 10, it is moved out of alignment with the other pallets and is returned by gravity to the wheel 6. At the same time the continuous movement of the sintering cake, which is indicated in the drawings by 11 carries it onto a supporting shelf 12 which 40 is in alignment with the bottoms of the pallets.

B represents as an entirety the furnace for smelting the sinter cake. This furnace comprises side and end walls 13, a bottom 14 45 and an arched roof 15. The various parts of the furnace may be formed of any suitable heat resisting materials which are adapted for use in connection with the ore to be treated.

50 In one end wall of the furnace there is provided an aperture 16 adapted to receive the end of the continually moving sinter cake 11. I prefer to so construct the conveyer 1 that the sinter cake will be fed into the furnace at a slight downward angle, the purpose of which will be hereinafter fully set forth. If desired, supporting ledges of fire brick may be formed to support the advancing sinter cake. I do not, however, 55 at present consider these ledges necessary and have not therefore shown them in the drawings.

The bottom of the furnace is adapted for the collection and retention of a bath of 60 matte or molten metal. A tap 17 is pro-

vided for the withdrawal of the metal from time to time. On top of the metal bath, there will collect a layer of slag consisting of silicious or other material. This layer of slag is formed either from material contained normally in the ore itself or it may be derived from fluxing materials mixed with the ore before it reaches the desulfurizing and sintering apparatus. If preferred, however, the fluxing materials can be separately introduced into the furnace by means of a hopper and chute, such as is indicated by 18.

19 is a slag-tap adapted for the occasional or continual removal of the slag. The tap 80 19 may discharge into a suitable slag car, such as indicated by 20. The tap is located at such an elevation that the slag will be maintained at a level somewhat above that of the inner end of the sinter cake 11. I 85 have found that, on account of its porous nature, the sinter cake is lighter than the slag and will consequently tend to float thereon. By submerging the inner end of the sinter cake its tendency to break by its 90 own weight is counteracted.

21 and 22 represent two sets of electrical contact devices arranged respectively above and below the moving sinter cake. These contact devices may be of any preferred 95 form, but for purposes of illustration I have shown them as comprising a series of 100 slideable spring-pressed rollers frictionally engaging with the surfaces of the cake. These contact devices are connected by means of a suitable conductor with one terminal of an electric generator. The other generator terminal is connected with a stationary electrode or contact plate 23 located 105 in the bottom of the furnace. This contact plate is preferably formed of carbon and by means of it electrical connection is established to the bath of metal in the furnace.

The sinter cake 11, on account of the metal 110 contained therein, forms an electric conductor having a rather high resistance, and the electric generator with which it is connected by means of the contacts 21 and 22 and the carbon plate 23 has sufficient voltage to 115 permit the completion of an electric connection between the end of the sinter cake and the molten metal beneath it, the current passing through the molten slag. Intense heat is generated by this action of the current in passing from the sinter cake to the molten metal and by means of it the end of the advancing cake is continually melted off. The current potential and the rate of movement 120 of the cake should be so adjusted relative to each other as to maintain the end of the solid cake at substantially the same part of the furnace. As the sinter cake is melted the pure metal is separated by gravity and unites itself with the mass of metal in the furnace. The slag and impurities float on top of the 125 130

metal and are withdrawn through the tap 19. The passage of the electric current through the sinter cake tends to heat it on account of the electrical resistance of the cake itself. It will be noted that the cake is subjected to four separate heating influences. First, the heat of sintering, which is retained as the cake passes into the furnace; second, the heat caused by the passage of the current through the sinter cake; third, the heat derived by conduction and radiation from the hot metal and slag; and fourth, the heat from the electric action at the end of the cake. It will, therefore, be noted that, 15 on account of the heating influences to which the cake is subjected before it reaches the smelting point, comparatively little additional heat need be generated at this point to cause melting.

20 I am aware that smelting by electrical means is a well known process and also that it has been proposed to carry out this process of electrical smelting by means of a current passing longitudinally through a continually 25 moving stream of ore. However, I believe myself the first to provide for an intensified electrical heating action to produce smelting at the end of the continually moving ore stream. Furthermore, so far as I am aware, 30 in previous processes the ore or other material to be treated has been supplied in fragmentary condition. By using my invention it is possible to agglomerate or sinter and smelt the ore by one continuous operation, 35 and on this account my improved process is carried out much more economically than those previously proposed. I do not desire, however, to limit my improved process to a single unitary operation, as in certain cases 40 it may be found possible or desirable to carry out the process by two distinct separate operations. First, the sinter cake may be formed either in long bars or in smaller fragments and afterward fed to an electrical furnace similar to that which I have described.

45 In fact, it is not absolutely necessary, so far as this invention is concerned, that the sinter cake be formed by means of the process, or of the apparatus which I have described.

50 One of the advantages incident to my improved process is that the sinter-electrode may be so made up previous to its entrance into the furnace that its chemical composition, including the necessary fluxes, will be 55 exactly right for the most economical and efficient smelting and for the formation of the correct chemical slag and other products. The quantity of sulfur in the case of sulfid ores or of carbon in the case of iron ores may be left such that the metal matte or regulus resulting from the smelting will be exactly what is desired. Another advantage is that the extremely intimate mixture of the ingredients of the sinter cake is conducive of 60 extraordinarily rapid smelting. In fact, the

chemical reactions of the sintering processes are similar to those of the smelting processes, and therefore the sinter cake may be considered as partly smelted before it enters the furnace.

70 I have shown and described the sinter cake as entering the furnace substantially horizontally. However, it may be found possible or desirable to feed the sinter cake vertically or at some oblique angle. It may also be possible in certain modifications of my process to feed the cake into the furnace on edge.

75 I do not limit myself to a single sinter-electrode and in a co-pending application entitled Apparatus for sintering and smelting ores, filed March 31, 1910, Serial No. 552,580, I have shown and described an apparatus for feeding two oppositely moving sinter-electrodes and forming an electric action between them.

80 I do not claim as part of my present invention the apparatus which I have shown and described. This apparatus is described and claimed in a copending application by me, entitled Apparatus for sintering and smelting ores, filed March 31, 1910, Serial No. 552,579.

85 Neither do I claim in this case the process of obtaining metal from ore which is initially in a fine condition which consists 90 in forming the ore in a relatively thin layer or stream, sintering the ore while in such layer, and introducing the sinter thus formed into a smelting furnace where it is smelted; as such process is made the subject of my aforesaid application No. 440,404, for process of sintering and smelting ores; nor do I here claim the process of treating porous metalliferous sinter by bringing it into intimate contact with molten slag that 95 is maintained at a temperature sufficient to cause smelting of the sinter, as that process is made the subject-matter of and claimed in my co-pending application No. 636,296, filed June 30, 1911.

100 What I claim is:—

105 1. The herein described process of sintering and smelting ore, which consists in sintering a layer of ore into a continuous sinter cake, continually moving the said cake away from the region of sintering, subjecting the cake intermediate its ends to the action of an electric current, and subjecting it at its advance end to the action of an electric current which passes from the 110 end of the cake to a relatively stationary conductor body, substantially as set forth.

115 2. The herein described process of sintering and smelting ore, which consists in sintering a layer of ore into a continuous sinter cake, continually moving the cake away from the region of formation and subjecting the said cake to the action of an electric current, the said current passing 120 through the cake and from the advance end 125 130 135 140 145 150 155 160 165 170 175 180 185 190 195 199

- of the cake to a relatively stationary electrode, substantially as set forth.
3. The herein described process of sintering and smelting ore, which consists in sintering a layer of ore into a continuous cake, and subjecting the said cake while it still retains the heat of sintering to the action of an electric current, the said current passing through the cake, and from the advance 70 end of the cake to a relatively stationary electrode, substantially as set forth.
4. The herein described process of sintering and smelting ore of the class adapted to be sintered by the combustion of materials contained therein, which consists in arranging the ore in a continually moving layer, igniting the layer to cause combustion and sintering, and subjecting the sintered layer to the action of an electric current, while it 75 still retains the heat of sintering, the said current passing through the cake, and from the advance end of the cake to a relatively stationary electrode, substantially as set forth.
5. The herein described process of sintering and smelting ore, which consists in forming a continuous cake of sintered ore, continually moving the cake away from the region of formation, smelting the advance 80 end of the said moving cake, and passing an electric current through the said cake intermediate its ends to raise the temperature thereof, substantially as set forth.
6. The herein described process of sintering and smelting ore, which consists in sintering a layer of ore into a continuous sinter cake, continually moving the cake away from the region of sintering, smelting the advance end of the said moving cake and 85 subjecting the cake intermediate its ends to a heating influence separate from the smelting means, substantially as set forth.
7. The herein described process of smelting and sintering ore, which consists in sintering a layer of ore into a continuous sinter cake, continually moving the cake away from the region of sintering, smelting the advance end of the moving cake and subjecting the cake intermediate its ends to a 90 plurality of independent heating influences each separate from the smelting means, substantially as set forth.
8. The herein described process of ore treatment, which consists in sintering a layer of ore into a continuous sinter cake, continually moving the said cake as it is formed away from the region of sintering, and passing an electric current through the said moving cake to raise the temperature thereof, substantially as set forth.
9. The herein described process of ore treatment which consists in sintering a layer of ore into a continuous sinter cake, causing relative movement between the cake and the region of sintering, and passing an electric 95 current through the said cake to raise the temperature thereof, substantially as set forth.
10. The herein described process of ore treatment, which consists in sintering a mass of ore causing relative movement between the ore mass and the region of sintering, and passing an electric current through the said mass while it retains the heat of sintering to further raise the temperature thereof, substantially as set forth.
11. The herein described process of treatment for ore of the class adapted to be sintered by the combustion of materials contained therein, which consists in arranging the ore in a continuously moving layer, igniting the layer to cause combustion and sintering, and subjecting the sintered layer to the action of an electric current, while the heat of sintering is retained, to further 100 raise the temperature thereof, substantially as set forth.
12. The herein described process of ore treatment which consists in arranging the ore in a continuously moving layer, subjecting the layer to a heating action and then passing an electric current through it, the said current passing through the layer and from the advance end of the layer to a stationary conductor body, substantially as set forth.
13. The herein described process of ore treatment which consists in continually forming a continuous homogeneous cake of material adapted to be smelted, causing the 105 said cake to be heated, continually moving the said cake away from the region of formation and passing an electric current through the advance part of the said moving cake, substantially as set forth.
14. The herein described process of sintering and smelting ore, which consists in continually forming a continuous layer of the ore, subjecting the layer to the action of heat to cause sintering, continually moving the ore away from the region of forming and sintering, subjecting the forward end of the sinter cake to a continual smelting action, and applying heat to the said layer at points intermediate the region of sintering 110 and the region of smelting, the said heat being derived independently of the heat of sintering and of the heat of smelting, substantially as set forth.
15. The herein described process of sintering and smelting ore masses containing combustible ingredients, which consists in continually forming a continuous layer of the ore, together with the said combustible ingredients, causing the combustion of the said 115 combustible ingredients within the ore mass whereby sintering is effected, continually moving the resulting sinter cake away from the region of sintering, subjecting the forward end of the sinter cake to a continual 120
16. The herein described process of sintering and smelting ore masses containing combustible ingredients, which consists in continually forming a continuous layer of the ore, together with the said combustible ingredients, causing the combustion of the said 125 combustible ingredients within the ore mass whereby sintering is effected, continually moving the resulting sinter cake away from the region of sintering, subjecting the forward end of the sinter cake to a continual 130

smelting action, and applying heat to the cake at points intermediate the region of sintering and the region of smelting, the said heat being derived independently of the heat of sintering and of the heat of smelting, substantially as set forth.

16. The herein described process of ore treatment which consists in continually forming a continuous layer of the ore, continually moving the said layer away from the region of formation, subjecting the layer to a heating action at points adjacent the region of formation, continually subjecting the forward end of the layer to a smelting action, and applying heat to the ore at points intermediate the region of initial heating and the region of smelting, the said heat being derived independently of the heat of the said initial action and of the heat of smelting, substantially as set forth.

17. The herein described process of sintering and smelting ore, which consists in continually forming a layer of the ore, continually moving the said layer away from the region of formation, subjecting the layer to heat at points adjacent the region of formation to cause sintering, subjecting the forward end of the sintering layer to a smelting action, and passing an electric current through the layer at points intermediate the region of sintering and the region of smelting to raise the temperature thereof, substantially as set forth.

18. The herein described process of sintering and smelting ore masses containing combustible ingredients which consists in forming a continuous layer of the ore, together with the said combustible ingredients, causing the combustion of the said combustible ingredients at points adjacent the region of formation to cause sintering, subjecting the forward end of the sintered layer to a smelting action, and passing an electric current through the layer at points intermediate the region of sintering and the region of smelting to raise the temperature thereof, substantially as set forth.

19. The herein described process of ore treatment, which consists in continually forming a continuous layer of the ore, continually moving the layer away from the region of formation, subjecting the layer to a heating action at points immediately adjacent the region of formation, subjecting the advance end of the said layer to a smelting action, and passing an electric current through the layer at points intermediate the region of the initial action and the region of smelting to raise the temperature of the layer, substantially as set forth.

20. The herein described process of sintering and smelting ore, which consists in continually forming a continuous layer of the ore, continually sintering the said layer into a continuous cake, continually moving the

cake away from the region of forming and sintering, continually subjecting the forward end of the cake to electric action to cause smelting, and applying heat to the said layer at points intermediate the region of sintering and the region of smelting electric action, the said heat being derived independently of the heat of sintering and of the heat of the smelting action, substantially as set forth.

21. The herein described process of sintering ore, which consists in continually forming a continuous layer of the ore, continually moving the layer away from the region of formation, applying heat to the layer at points immediately adjacent the region of formation to cause sintering, continually subjecting the forward end of the resulting sinter cake to electric action to cause smelting, and applying heat to the said layer at points intermediate the region of sintering and the region of the electric smelting action, the said heat being derived independently of the heat of sintering and of the heat of smelting, substantially as set forth.

22. The herein described process of sintering and smelting ore masses containing combustible ingredients which consists in continually forming a continuous layer of the ore together with the said combustible ingredients, causing combustion of the said combustible ingredients to effect sintering, continually moving the resulting sinter cake away from the region of formation and sintering, subjecting the forward end of the sinter cake to electric action to cause smelting, and applying heat to the cake at points intermediate the region of sintering and the region of smelting, the said heat being derived independently of the heat of sintering and the heat of smelting, substantially as set forth.

23. The herein described process of ore treatment which consists in continually forming a continuous layer of the ore, continually moving the layer away from the region of formation, subjecting the layer at points immediately adjacent the region of formation to a heating action, continually subjecting the forward end of the layer to electric action to cause smelting, and applying heat to the layer at points intermediate the region of the initial heating action and the region of smelting action, the said heat being derived independently of the heat of the initial heating action and of the heat of smelting, substantially as set forth.

24. The herein described process of sintering and smelting ore masses containing combustible ingredients, which consists in continually forming a layer of the ore together with the combustible ingredients, causing combustion of the said combustible ingredients at points adjacent the region of formation to effect sintering of

- the layer, continually moving the resulting sinter cake away from the region of forming and sintering, passing an electric current through the moving cake at points beyond the region of sintering, and subjecting the forward end of the cake to electric action to cause smelting, substantially as set forth.
25. The herein described process of ore treatment which consists in continually forming a continuous layer of the ore, continually moving the layer away from the region of formation, subjecting the layer to a heating action at points immediately adjacent the region of formation, passing an electric current through the layer at points beyond the region of the initial heating action, and subjecting the forward end of the layer to electric action to cause smelting, substantially as set forth.
26. The herein described process of sintering and smelting fine ore which consists in forming the ore into relatively thin and substantially uniformly porous sinter and subsequently subjecting such sinter within a furnace to a smelting heat produced by the passage of a current of electricity, and finally separating the metallic parts of the ore from the remaining components thereof.
- 30 27. The herein described process of recovering the metal from metal-bearing material that is initially in a finely divided condition, which consists in agglomerating the said material into a rigid mass that is highly and uniformly porous throughout,
- 35

introducing this mass endwise into the free space of a smelting furnace above a fused bath formed by the smelting of the material being treated, causing a current of electricity to pass from the end of the said rigid mass of material into the bath and thereby smelting the former and maintaining the latter in fused condition, and finally separating the metallic parts of the bath from the other components thereof.

28. The herein described process of recovering metal from metal-bearing material that is initially in a finely divided condition, which consists in agglomerating the said material into a rigid mass that is highly and uniformly porous throughout, introducing this mass endwise into a smelting furnace above and across a fused bath formed by the smelting of the material being treated, causing the end of the mass to come in contact with the said fluid bath whereby it is partially supported thereby, causing a current of electricity to pass through the said rigid mass of material and from it into the bath, whereby the former is smelted and the latter maintained in fluid condition, and finally separating the metallic from the other component parts of the bath.

In testimony whereof I affix my signature, in presence of two witnesses.

ARTHUR S. DWIGHT.

Witnesses:

H. J. STEHLI,  
C. M. STANLEY.